

Patented June 17, 1941

2,246,085

# UNITED STATES PATENT OFFICE

2,246,085

## COMPOSITION AND PROCESS FOR SOFTENING LEATHER, PAPER, AND TEXTILE MATERIALS

Luther B. Arnold, Jr., Wilmington, Del., assignor to E. I. du Pont de Nemours & Company, Wilmington, Del., a corporation of Delaware

No Drawing. Application February 23, 1938,  
Serial No. 192,162

5 Claims. (Cl. 134—11)

This invention relates to treating agents for fibrous materials and to processes of treating such materials. More particularly it relates to compositions for softening leather, paper and textile materials and to processes therefor. Still more particularly it relates to textile treating compositions which contain high molecular weight sulfuric acid esters and urea. The invention also relates to processes of preparing such compositions.

This invention has for an object the production of chemical compositions which are useful in softening leather, paper, textile and related materials. A further object is the production of chemical compositions which have good softening action upon leather, paper and textile materials and render the same soft and pliable to the touch. A still further object is the preparation of softening compositions which render textile, leather and paper materials treated therewith pleasing in appearance, of good odor, and unchanged in color. Other objects include new leather, paper and textile treating processes and a general advancement in the art.

I have found that when urea is used in combination with long chain alcohol sulfate ester salts in certain proportions and incorporated in aqueous solutions for treating leather, paper and textile materials, they impart a novel finish to the same. The alcohol sulfate ester compositions containing certain proportions of urea when used in solution for treating fibrous materials such as cotton, hemp, jute, linen, wool, silk, regenerated cellulose, cellulose derivatives, e. g. cellulose acetate and wood pulp render the same when in filament, thread, skein, yarn or sheet form, soft and smooth to the touch and in general more pleasing in appearance.

The above and other objects are accomplished by the following invention which in one embodiment comprises adding to an aqueous treating bath for fibrous materials from 1 to 50 parts of urea per part of long-chain alcohol sulfate ester or per part of softening agent based upon the long-chain alcohol sulfate esters as determined on a dry basis. Thus, while the alcohol sulfates form an essential part of the composition other softening agents may be incorporated in the compositions such as the compounds prepared by sulfonating long chain aliphatic and cycloaliphatic hydrocarbons such as the hydrocarbons derived from petroleum.

The long-chain alcohol sulfate ester salts used according to the present invention may contain from 8 to 20 carbon atoms in the chain. They may be prepared by partially or completely sulfating long chain aliphatic alcohols and neutralizing the sulfuric acid esters with alkali metal bases. The preparation of these products is described in the chemical literature and is well

known to the art. Suitable salts of the alcohol sulfuric acid esters and their preparation are described in Bertsch Patents Nos. 1,968,794, 1,968,797 and 1,993,431. The products may also comprise the mixtures obtained by treating unsaturated long-chain alcohols with acid anhydrides, such as acetic anhydride prior to sulfation.

The invention will be further illustrated but is not intended to be limited by the following examples:

### Example I

An aqueous solution is prepared containing 0.2% of sodium cetyl sulfate and 0.4% of urea. It is heated to 50° C. and applied to fabrics made from regenerated cellulose or cotton by passing them through the solution. After drying the fabrics are found to have a very smooth soft surface in addition to being pliable.

### Example II

A solution is prepared containing 0.5% by weight of the sodium salt of the product obtained by the conjoint sulfation of stearyl alcohol and petrolatum and 0.5% by weight of urea. Taffeta fabrics woven from regenerated cellulose and broadcloth fabrics woven from cotton after being treated in this solution at 40–60° C. and dried are found to possess a very smooth velvety surface as well as being soft and pliable. Many other types of fabrics from all known textile fibers, synthetic or natural, may be treated in a similar manner. For example, crepe fabrics from artificial silk, crepe fabric from artificial silk and cotton, printed dress fabrics from cotton and draperies from artificial silk and from cotton may be treated with urea and alcohol sulfate esters or softening agents based on alcohol sulfate esters in order to enhance their finish.

### Example III

Paper is treated by padding onto it a solution containing 0.1% by weight of sodium cetyl sulfate and 2.0% by weight of urea. After drying the paper has a soft, smooth surface.

The following examples illustrate the preparation of alcohol sulfate ester salts and softening agents containing urea:

### Example IV

Nineteen and three-tenths parts by weight of cetyl alcohol are sulfated with 7.6 parts by weight of chlor sulfonic acid with agitation of the mass over a period of 30–40 minutes with the temperature maintained at 55–65° C. The mass is then stirred for 4 to 5 minutes to allow the reaction to come to an end. Sixty and three-tenths parts by weight of 5.4% sodium hydroxide at 30° C. are added to the reaction mass slowly during stirring. Fifty parts by weight of urea are then added, the

temperature is raised to 45-50° C. and the mass is stirred until it is homogeneous.

The product is a homogeneous, white paste in appearance. It emulsifies readily in warm water with simple agitation.

The sulfation may be also carried out to obtain still less complete sulfation of the aliphatic alcohol in order to change the finishing effect of the product. Textiles, leather and paper may be treated with this product following the procedure of Examples I, II and III.

*Example V*

Nineteen and three-tenths parts by weight of stearyl alcohol and 12.8 parts by weight of refined petrodatum (M. P. range 40-50° C.; Iodine No. 10-20) are melted together and 7.6 parts of chlor sulfonic acid (92% by theory on weight of stearyl alcohol) are added during agitation of the mass over a period of 30-40 minutes with a temperature maintained at 55-65° C. The mass is then stirred for 3 to 4 minutes to allow the reaction to come to an end. Sixty and three-tenths parts by weight of 5.4% sodium hydroxide at 30° C. are added to the reaction mass slowly during stirring. One hundred and thirty-three parts by weight of urea are added. The temperature is brought to 50-60° C. and the mass is stirred until homogeneous.

The product is a homogeneous, white paste in appearance. It emulsifies readily in warm water with simple agitation and dilute emulsions even up to 5% will not separate after 10-20 minutes boiling or even while cooling from the boiling point.

In place of the specific alcohols of Example V, other alcohols having from 8 to 20 carbon atoms, preferably normal straight chain alcohols or mixtures, may be used. Thus, dodecyl, myristyl, cetyl, oleyl or mixtures of the same may be substituted for the stearyl alcohol. The alcohols may be pure or of the crude or technical type, or may be mixtures.

Likewise, other hydrocarbon materials may be substituted for the refined petrodatum of Example V. Light mineral oils of 50 to 100 Saybolt units of viscosity at 100° F., heavy mineral oils of 100 to 300 Saybolt units of viscosity at 100° F., petrodatum wax, paraffin wax or mixtures of these materials may be used. Mixtures of petrodatum with the mineral oils and/or paraffin wax give excellent results.

Dry products which represent an important embodiment of this invention may be prepared in various ways. A sulfation product may be dried immediately after neutralization and the dry material ground with crystalline urea. The neutralized product resulting from the sulfation may be dried after the addition of urea and then ground to a stable powder or it may be dried upon a drum dryer to form a flake product.

Products which have been prepared by sulfating fatty alcohols with sulfuric acid containing up to 30% of its weight of urea do not have any greater softening power than the product after removing the urea therefrom does. I have found that if a material amount of urea is added to such products so that the urea is present in 1 to 50 parts per part of alcohol sulfate and preferably from 3 to 10 parts, the softening power of the product is greatly increased and a novel finishing effect is produced upon fibrous materials treated therewith. The urea may be added

to a solution or to the dry product in the manner above described.

Similarly, sulfation products which have been neutralized by treatment with urea can be made into excellent textile treating compositions by adding sufficient urea to bring the amount of urea to alcohol sulfate or agent based upon alcohol sulfate to 1 to 50 and preferably 3 to 10 parts by weight per part of the latter. The additional urea may be added to a solution or to a dry product according to the procedure set forth above.

The products (e. g., those illustrated in Examples IV and V) may be applied to leather, paper or textiles at concentrations varying over a wide range. Concentrations varying from 0.05 to 5% as illustrated in Examples I to III represent a practical range.

This invention possesses the advantages that softening and textile treating compositions may be quickly and economically prepared. The products may be used alone or in conjunction with other softening agents especially those of the alcohol sulfate type. The compositions may be used for after treating bleached, dyed and printed textile products. The compositions may also be used with weighting and loading agents such as starches, starch derivatives and by-products, and mineral weighting agents. Stable solutions with calcium and magnesium salts may be prepared. Hydroscopic agents such as glycerine and glycols may be employed in conjunction with my compositions.

The compositions may be used in the dyebath as a dispersing and softening agent for use in dyeing with a wide range of types of dyestuffs. They are not compatible with the basic colors, however. They may be used along with bleaching agents in a bleaching operation.

As many apparently widely different embodiments of this invention may be made without departing from the spirit and scope thereof, it is to be understood that I do not limit myself to the specific embodiments thereof, except as defined in the appended claims.

I claim:

1. A dry powder consisting of 1 to 50 parts of urea and 1 part of a mixture obtained by the conjoint sulfation of crude octadecyl alcohol and petrodatum and neutralization with a water soluble base.

2. The process which comprises treating fibrous materials in an aqueous bath consisting of water and a small amount of a mixture consisting of 1 to 50 parts of urea and 1 part of a mixture obtained by the conjoint sulfation of a normal primary aliphatic alcohol of at least 8 carbon atoms and a higher petroleum hydrocarbon.

3. An aqueous textile treating solution containing a small amount of a mixture consisting of 1 to 50 parts of urea and 1 part of a mixture obtained by the conjoint sulfation of a normal primary aliphatic alcohol of at least 8 carbon atoms and a higher petroleum hydrocarbon.

4. An aqueous paste comprising 1 to 50 parts of urea and 1 part of a mixture obtained by the conjoint sulfation of a normal primary aliphatic alcohol of at least 8 carbon atoms and a higher petroleum hydrocarbon.

5. An aqueous paste comprising 1 to 50 parts of urea and 1 part of a mixture obtained by the conjoint sulfation of stearyl alcohol and refined petrodatum.

LUTHER B. ARNOLD, JR.